

(No Model.)

H. W. JOHNSON.  
CHAIR SEAT.

No. 552,840.

Patented Jan. 7, 1896.

Fig. 1.



Fig. 3.



Inventor

Henry W. Johnson.

Witnesses  
John A. Heiden, Fig. 2.  
John Washington Miller, Fig. 3  
By Baldwin, Dawson & Wright  
Attorneys

# UNITED STATES PATENT OFFICE.

HENRY W. JOHNSON, OF MICHIGAN CITY, INDIANA.

## CHAIR-SEAT.

SPECIFICATION forming part of Letters Patent No. 552,840, dated January 7, 1896.

Application filed February 12, 1895. Serial No. 538,104. (No model.)

*To all whom it may concern:*

Be it known that I, HENRY W. JOHNSON, a citizen of the United States, residing at Michigan City, in the county of Laporte and State 5 of Indiana, have invented certain new and useful Improvements in Chair-Seats, of which the following is a specification.

My invention more especially relates to chair-seats comprising woven-cane fabric in 10 their construction; but such fabric has usually been woven plain. Sometimes it is twilled, but has never been woven, so far as my knowledge extends, with ornamental figures.

15 The principal object of my invention is to make such seats of figured fabric; but this involves special difficulties to be overcome. The figuring of the fabric involves the passage of some threads over several others, and 20 the cane being stiff and non-elastic these overlapping or floating portions tend to protrude unduly, thus injuriously affecting both the appearance and the durability of the fabric. In order to obviate these objections and to 25 secure an attractive, durable, and efficient seat, I weave the cane into the desired figure or pattern and then secure the overlapping, protruding, or floating portions to the other threads of the fabric by cement, glue, or paste, 30 so as to obtain a uniform surface. I further strengthen the fabric by cementing, gumming, or pasting a fabric—such, for instance, as stout canvas—to the under side of the cane fabric and also to the floating portions of the 35 cane. This backing or foundation aids materially not only in giving body to the seat, but also in holding the strands or threads of the cane in place.

40 The fabric which I have described as especially adapted for chair-seats is also well adapted for use as a floor covering in the place of ordinary matting.

In the accompanying drawings, Figure 1 is 45 a plan view of a portion of a close-woven cane fabric with a design woven therein according to my invention, showing also a canvas backing to which the cane fabric is secured. Fig. 2 is a detail view, on an enlarged scale, showing how the threads of the fabric are 50 interwoven. Fig. 3 shows a cross-section on the line 3 3 of Fig. 2.

The cane fabric A may be woven in any

suitable way, either by hand or by machinery, and is twilled as shown to form the desired figures. In this instance a series of diamond-shaped figures, one within the other, is formed. Where the fabric is twilled there are floating portions b, which tend to stand up from the surface or upper plane of the fabric and form an objectionable rough surface; but I employ 55 paste, glue, or cement to secure these floating portions to the threads of the fabric below them, and by applying suitable pressure to the fabric when thus cemented a smooth and even surface may be obtained. 60

65 As an additional security I attach to the under side of the cane fabric a sheet C, of suitable material, such as duck or canvas. This may be covered on the side adjacent to the fabric A with cement, glue, or paste, and 70 pressure is applied to cause the cement to connect the sheet C not only with the threads of the body of the fabric, but also and especially with the floating portions of the threads.

75 It will be observed by reference to Fig. 3 that the cement z is arranged between the overlapping portions of the warp and weft threads, and also is arranged between the sheet C and the adjoining threads of the fabric A. 80

Any suitable cement, paste, or glue may be employed, but preferably such as is not affected by moderate heat or by dampness.

In the manufacture of the fabric embodying my invention, the figured cane cloth is 85 first woven by machinery and the canvas backing is covered with a thick layer of paste or cement. The cane cloth is laid on the cemented side of the canvas, and then heavy pressure is supplied to cause the cement to 90 pass through the interstices of the cane fabric, permeating the spaces between the warp and weft threads and also filling the spaces between the floating portions of the warps and the canvas. The cement is allowed to partially harden and then the front face of the fabric is sponged or washed off to remove the exposed cement. Additional pressure may then be employed to flatten out the fabric and more securely unite the cane to the canvas 95 after the cement is dry. The fabric is then 100 ready for use.

I claim as my invention—

A fabric adapted for chair seats, &c., com-

prising a woven figured fabric of cane or rattan, the overlapping or floating portions of the warps being cemented to the underlying wefts, and a backing of canvas, or similar material, cemented to the adjacent portions of the warps and wefts, and also to the floating portions of the warps, substantially as described.

In testimony whereof I have hereunto subscribed my name.

HENRY W. JOHNSON.

Witnesses:

HENRY B. MORRIS,  
EDMUND MORRIS.